

## UNITED STATES PATENT OFFICE

2,113,653

## CELLULOSE DERIVATIVE COMPOSITIONS

James Karr Hunt and George Henry Latham,  
Wilmington, Del., assignors to E. I. du Pont  
de Nemours & Company, Wilmington, Del., a  
corporation of Delaware

No Drawing. Original application July 15, 1933,  
Serial No. 680,656. Divided and this applica-  
tion April 24, 1936, Serial No. 76,261

8 Claims. (Cl. 106—40)

This invention relates to cellulose derivative compositions containing non-drying and semi-drying fatty bodies and agents for inhibiting rancidity development thereof and, more particularly, to cellulose nitrate compositions employed in the manufacture of artificial leather, and the like.

Numerous compounds have heretofore been suggested as agents for inhibiting rancidity in non-drying and semi-drying fatty bodies and a few compounds have been suggested as rancidity inhibiting agents for use in cellulose derivative compositions. However, the heretofore suggested compounds are usually either unsatisfactory as regards the inhibition of rancidity, or they seriously affect the initial color of cellulose derivative "dopes", cause discoloration of films deposited from the dopes on exposure to the sunlight, render such films sensitive to water, cause spotting or fading of the color, or else have an objectionable odor. Most of the prior art has related only broadly to the inhibition of rancidity in oils and has given no indication of the suitability of suggested compounds for use in cellulose derivative dopes. The mere suggestion of a compound as a rancidity inhibitor for oils is of practically no value toward the selection of an agent having that unique combination of properties which will make it satisfactory for use in cellulose derivative dopes, particularly white or light colored cellulose nitrate compositions.

An object of the present invention is to provide improved cellulose derivative compositions for coating artificial leather, and the like, containing a non-drying or semi-drying fatty body and a rancidity inhibiting agent therefor. A further object is to provide such compositions containing a non-drying or semi-drying fatty body having a tendency to become rancid and having, in the raw state, a normal iodine number below 135 and a rancidity inhibiting agent therefor which will not affect the initial color of the composition, cause discoloration of films deposited therefrom on exposure to the sunlight, render said films sensitive to water, cause spotting or fading of the color, or have an objectionable odor. Other objects of the invention will be apparent from the description given hereinafter.

The above objects are accomplished according to the present invention by incorporating in a cellulose derivative coating composition containing a non-drying or semi-drying fatty body having a tendency to become rancid and having, in the raw state, a normal iodine number below 135,

but preferably below 120, an agent selected from the group consisting of aryl boric acids.

Among the aryl boric acids found particularly adapted for the purpose of the present invention are:



phenyl boric acid



p-tolyl boric acid

These compounds are expressed comprehensively by the formula



where R is any monovalent organic radical joined to the boron atom through an aromatic carbon atom, and R<sub>1</sub> is hydroxyl or a monovalent organic radical joined to boron through an aromatic carbon atom. Other suitable boric acids of this general formula are alpha-naphthyl boric acid, di-p-anisyl boric acid, di-beta-naphthyl boric acid, and p-carboxy-phenyl boric acid.

It has been found that the above class of compounds has properties which are remarkably well adapted for using said compounds in cellulose derivative compositions containing non-drying and semi-drying oils and other fatty bodies tending to become rancid. That is, these compounds are effective for inhibiting rancidity in compositions containing non-drying and semi-drying fatty glycerides which have a tendency to become rancid and have, in the raw state, a normal iodine number below 135 and particularly in such oils having an iodine number below 120; do not give an objectionable odor to the compositions, do not give rise to objectionable discoloration of the compositions, and do not render the compositions sensitive to water.

In order to test the effect of our compounds in coating compositions or "dopes" employed in the manufacture of artificial leather a representative "dope" was prepared as follows:

|                                            | Parts (by weight) |    |
|--------------------------------------------|-------------------|----|
| Cellulose nitrate                          | 11.5              |    |
| Castor oil                                 | 18.0              | 50 |
| Pigment                                    | 11.0              |    |
| Ethyl alcohol                              | 36.0              |    |
| Ethyl acetate                              | 23.5              |    |
| Inhibitor (2% based on castor oil content) | 0.36              | 55 |

The cellulose nitrate was dispersed in a mixture of the ethyl alcohol and ethyl acetate, and the pigment ground in a portion of the castor oil. The remain castor oil was mixed with the cellulose nitrate dispersion, following which the pigment in oil was added and the whole thoroughly mixed. The inhibitor was added as an alcoholic solution along with the pigment in oil.

In order to determine the effect of the inhibitors on the color of a dope of this type, the pigment consisted of lithopone or a mixture of 98.5% lithopone and 1.5% ultramarine blue. The compositions containing these pigments, because of their white or pale blue color, are highly susceptible to discoloration by inhibitors of the wrong type, and also lend themselves well to observations for "water spotting".

By the term "water spotting" is meant a color change, such as fading, which takes place when the artificial leather is brought into contact with water.

A suitable procedure for testing rancidity inhibitors in compositions of the above type follows: Various dopes are applied to pieces of fabric in the usual manner for making artificial leather, which treated pieces of fabric are then subjected to the following tests. A sample of treated fabric of standard size (e. g., 2" x 5") is placed in a small glass-stoppered flask and stored at a temperature of about 65°C. The various bottles are opened daily, or at other suitable intervals, and, from the odor emitted, a determination as to when rancidity develops is made.

The various pieces of treated fabric are subjected to exposure to the light from a glass-enclosed carbon arc for 16 hours and the change in color is compared with that of a sample of cloth treated with the same dope containing no inhibitor, in order to determine the effect of the inhibitors on the color change caused by exposure to sunlight.

A small strip of each sample of the treated fabric is immersed in water for 2 days and then dried. A comparison of the samples will disclose the effect of the inhibitors on water spotting or color change caused by the water.

The following table discloses the results obtained by the use of certain of our preferred inhibitors when incorporated in an artificial leather prepared as above described. In each case, 2% of the inhibitor, based on the castor oil, was employed.

Table

| 55 | Inhibitor          | Days for rancidity development* | Color changes | Water spotting |
|----|--------------------|---------------------------------|---------------|----------------|
| 60 | None               | 7                               | None          | None           |
|    | Phenyl boric acid  | 100+                            | None          | None           |
|    | p-Tolyl boric acid | 100+                            | None          | None           |

\* The "+" sign indicates no rancidity after number of days shown.

None of these compounds had any effect on the initial color of the artificial leather or gave the artificial leather an objectionable odor. In fact, all of the aryl boric acids are substantially odorless.

Cellulose propionate, cellulose acetate, ethyl cellulose, dodecyl cellulose, crotyl cellulose, benzyl cellulose, and similar cellulose derivatives may be employed instead of nitro-cellulose in cellulose derivative compositions comprising the non-drying or semi-drying oil, together with an inhibitor as above described.

In the above tests two percent of the inhibitor, based on the oil, has been employed. However, it is not necessary to employ these specific amounts, as larger or smaller proportions of the inhibitor may be used to advantage. The proportion of inhibitor will depend upon the particular type of composition, and especially the kind of oil used. It is practically never necessary to use more than 5% of inhibitor, based on the oil, and in some cases as little as 0.25% is useful. The percent of inhibitor is given by weight and not by volume.

The inhibitors have been disclosed specifically in coating compositions for dopes such as are generally used in the manufacture of artificial leather, said coating compositions containing castor oil. However, the inhibitors are adapted to be employed in other types of cellulose derivative compositions containing non-drying and semi-drying fatty bodies which have a tendency to become rancid and have, in the raw state, a normal iodine number below 135, or in such products when employed for other purposes. For example, the inhibitors of the present invention may be employed in cellulose derivative compositions containing resins and softeners derived from the various fatty acid glycerides.

Among the non-drying and semi-drying oils which may be treated satisfactorily with the inhibitors of the present invention, are olive oil, rapeseed oil, codliver oil, corn oil, peanut oil, cocoanut oil, cottonseed oil, palm oil, neat's-foot oil, butter fat, lard, beef tallow, wool fat, and the like. These oils, fats, and tallow may be raw or may have been previously subjected to various treatments, such as blowing with air at elevated temperatures, simple heat treatments, and the like, or the oils may be employed in making resins and softeners for use in artificial leather and similar compositions. Accordingly, the expression "non-drying and semi-drying bodies having a tendency to become rancid and having, in the raw state, a normal iodine number below 135", as used in the claims, is intended to include bodies of a resinous, oily, or waxy nature, having an iodine number below 135, which tend to become rancid with exposure to the atmosphere. Glycerol esters are most liable to rancidification; hence this invention is most concerned with such esters. However, the present inhibitors can also be added with advantage to other fatty acid esters, such as those of ethyl alcohol, butyl alcohol, mixtures of higher aliphatic monohydric alcohols, ethoxyethyl alcohol, ethylene glycol, propylene glycol, diethylene glycol, pentaerythritol, benzyl alcohol, et cetera. Fatty glycerides to which the present inhibitors can be added with especial advantage are those given in International Critical Tables Volume II, pages 201-205, under General Index Numbers 0.5-51 and 95-149 inclusive. The terminology used in the claims, referred to above, is intended to include all the above monohydric or polyhydric alcohol esters.

This is a division of our copending application Serial No. 680,656, filed July 15, 1933.

While certain compounds of general classes and certain fatty bodies employed in particular compositions have been disclosed, it is to be understood that other compounds of the same class may be employed for treating other fatty bodies of the type described, and the proportions and the constituents of the compositions in which they are employed may be widely varied without departing from the spirit of the invention. Accordingly, the scope of the invention is to be

limited solely by the appended claims construed as broadly as permissible in view of the prior art.

We claim:

1. A composition comprising a cellulose derivative, a fatty substance of the group consisting of non-drying and semi-drying fatty glycerides having a tendency to become rancid and having, in the raw state, a normal iodine number below 135, and, as a rancidity inhibitor therefor, a small percent of an aryl boric acid, based on the fatty substance.
2. A composition comprising a fatty substance of the group consisting of non-drying and semi-drying fatty glycerides having a tendency to become rancid and having, in the raw state, a normal iodine number below 135 and, as a rancidity inhibitor therefor, an aryl boric acid in a small percent based on the fatty substance.
3. A composition comprising a fatty substance of the group consisting of non-drying and semi-drying fatty glycerides having a tendency to become rancid and having, in the raw state, a normal iodine number below 135 and, as a rancidity inhibitor therefor, phenyl boric acid in a small percent based on the fatty substance.
4. A composition comprising a cellulose derivative, a fatty substance of the group consisting of non-drying and semi-drying fatty glycerides having a tendency to become rancid and having, in the raw state, a normal iodine number below 135, and, as a rancidity inhibitor therefor, a small percent of phenyl boric acid, based on the fatty substance.
5. A composition comprising a fatty substance of the group consisting of non-drying and semi-drying fatty glycerides having a tendency to become rancid and having, in the raw state, a normal iodine number below 135 and, as a rancidity inhibitor therefor, a tolyl boric acid in a small percent based on the fatty glyceride.
6. A composition comprising a fatty substance of the group consisting of non-drying and semi-drying fatty glycerides having a tendency to become rancid and having, in the raw state, a normal iodine number below 135 and, as a rancidity inhibitor therefor, p-tolyl boric acid in a small percent based on the fatty glyceride.
7. A composition comprising a fatty substance of the group consisting of non-drying and semi-drying fatty glycerides having a tendency to become rancid and having, in the raw state, a normal iodine number below 135 and, as a rancidity inhibitor therefor, a naphthyl boric acid in a small percent based on the fatty glyceride.
8. A composition comprising a fatty substance of the group consisting of non-drying and semi-drying fatty glycerides having a tendency to become rancid and having, in the raw state, a normal iodine number below 135 and, as a rancidity inhibitor therefor, alpha-naphthyl boric acid in a small percent based on the fatty glyceride.

30

JAMES KARR HUNT.  
GEORGE HENRY LATHAM.